

## UNITED STATES PATENT OFFICE

FERNANDO SOMOZA VIVAS, OF BRONXVILLE, NEW YORK

## PROCESS OF MANUFACTURE OF WALL BOARD, PRESSBOARD, AND THE LIKE

No Drawing.

Application filed December 3, 1929. Serial No. 411,387.

The invention relates to the manufacture of cellulosic fibre materials such as wall-board, pressboard, paper or the like and has as an object the provision of a process for producing a superior product.

It is a further object of the invention to provide a process of manufacturing heavily compressed material of cellulosic fibres, as pressboard, wherein a superior product may be produced with less pressure than that heretofore required.

It is a further object of the invention to provide a process of manufacturing the material of the character described using a novel form of binder to increase the coherence of the fibres.

It is a further object of the invention to provide a process of the character referred to wherein fireproofing materials in accordance with the disclosures of my co-pending applications, Serial Numbers 407,280 and 407,281 filed November 14, 1929, may be added to the binder provided by the invention so as to produce a fireproof material by the steps of the process.

Further objects of the invention will appear from the following description of illustrative embodiments of the invention.

In furtherance of the objects of the invention the pulp of which the material is to be manufactured is prepared in the usual manner with the addition of a solution including dextrine to the water in which the pulp is beaten. The amount of dextrine should be such as to provide a specific gravity of the solution in the beater, disregarding the fibres, of from 18° Bé. at 100° F. temperature to 21° Bé. at 200° F. temperature depending upon the material being manufactured as will be described below.

In the manufacture of porous wallboard or paper a lower specific gravity and temperature range is preferable but in the manufacture of highly compressed material as pressboard a higher specific gravity should be used. After the pulp has been prepared by beating with the solution described, the material may be formed into a sheet of wallboard or paper in the usual manner.

When pressboard is to be manufactured, it

has been found, contrary to all expectations, that the necessary pressure and temperature at which the material must be maintained during the pressure is very greatly reduced by the use of the materials described.

In the manufacture of a certain product of pressboard as heretofore carried out it has been necessary to press the material at from 500 to 600 pounds per square inch maintaining a temperature of from 350° F. to 400° F. while the pressure is applied. In accordance with the process of the invention it is found that an equally good or superior product may be secured by a pressure of from 150 to 200 pounds per square inch and that a temperature of from 212° F. to 225° F. is sufficient. Because of the lessening of the required pressure and temperature pressboard may be manufactured very much more economically than heretofore.

A modified form of binder containing dextrine which is found preferable for some purposes is described in my application Serial Number 407,281 above referred to and may be prepared as follows:

Substantially forty parts of starch are boiled with substantially sixty parts of glycerine until a transparent mass is produced. To the hot materials substantially 100 parts of alcohol are added and stirred with the mass to produce a solution thereof and to cause a cooling of the resultant solution. The alcohol may be either methyl or ethyl alcohol and the ethyl alcohol may be that usually sold as denatured alcohol prepared in accordance with any standard formula. The thus prepared solution may be substituted for the plain dextrine solution above referred to to provide a solution for use in the beater of the specific gravity described.

If it is desired to produce fireproof material the fireproofing materials of the above-mentioned co-pending applications may be added to the solution as described, utilizing substantially 1 pound 8 ounces of magnesium sulphate, 4 ounces borax, 4 ounces ammonium sulphate, 1.6 ounces alco-glycero-dextrine solution above described; or 1½ pounds of magnesium chloride, 4 ounces of boric acid, 100

55

60

65

70

75

80

85

90

95

4 ounces ammonium chloride with 1.6 ounces of the plain dextrine solution.

Minor changes in the steps of the process or in the quantities of ingredients used may 5 be made within the scope of the following claims without departing from the spirit of the invention.

I claim:

1. The process of producing a sheet of 10 felted cellulosic fibres which comprises beating the pulp in the preparation thereof with a solution comprising dextrine and forming a sheet from the thus prepared material.
2. The process of producing a sheet of 15 felted cellulosic fibres which comprises beating the pulp in the preparation thereof with a solution of the herein described alco-glycero-dextrine solution and forming a sheet from the thus prepared pulp.
3. The process of producing pressboard 20 which comprises beating a pulp of cellulosic fibres in a solution including dextrine, forming a sheet from the thus prepared pulp, and subjecting the sheet to pressure to express 25 the moisture and to produce a dense body of felted and compressed fibres.
4. The process of producing pressboard which comprises beating a pulp of cellulosic fibres in a solution including dextrine, forming 30 a sheet from the thus prepared pulp, and subjecting the sheet to pressure and heat to express moisture and set the fibres whereby to produce a dense body of felted fibres.
5. The process of producing pressboard 35 which comprises beating a pulp of cellulosic fibres in a solution including dextrine, forming a sheet from the thus prepared pulp, compressing the sheet at a pressure of substantially 200 pounds per square inch and subjecting the sheet while under pressure to 40 a temperature of substantially 225° F. whereby to set the sheet and produce a dense body of felted fibres.
6. The process of producing fireproof 45 pressboard which comprises beating a pulp of cellulosic fibres in a solution comprising the herein described alco-glycero-dextrine solution, magnesium and ammonium chlorides and boric acid, forming a sheet from 50 the thus prepared pulp, subjecting the sheet to a pressure of substantially 200 pounds per square inch and to a temperature of substantially 225° F. while held under pressure whereby to compress and set the fibres to 55 produce a dense fireproof body of felted fibres.

FERNANDO SOMOZA VIVAS.